



US007645560B1

(12) **United States Patent**  
**Iftime et al.**

(10) **Patent No.:** **US 7,645,560 B1**  
(45) **Date of Patent:** **Jan. 12, 2010**

(54) **INKLESS REIMAGEABLE PRINTING PAPER AND METHOD**

(75) Inventors: **Gabriel Iftime**, Mississauga (CA); **Gerald A. Domoto**, Briarcliff Manor, NY (US); **Tyler B. Norsten**, Oakville (CA); **Kentaro Morimitsu**, Mississauga (CA); **Paul F. Smith**, Oakville (CA); **Peter M. Kazmaier**, Mississauga (CA); **Gaetano J. Lavigne**, Oakville (CA); **Eric J. Shrader**, Belmont (CA); **Stephan V. Drappel**, Mississauga (CA)

(73) Assignee: **Xerox Corporation**, Norwalk, CT (US)

(\*) Notice: Subject to any disclaimer, the term of this patent is extended or adjusted under 35 U.S.C. 154(b) by 0 days.

(21) Appl. No.: **12/206,136**

(22) Filed: **Sep. 8, 2008**

(51) **Int. Cl.**

**G03F 7/00** (2006.01)

**G03F 7/004** (2006.01)

(52) **U.S. Cl.** ..... **430/270.1**; 430/19; 430/138; 430/270.15; 430/945; 430/962

(58) **Field of Classification Search** ..... 430/19, 430/138, 270.1, 270.15, 345, 962

See application file for complete search history.

(56) **References Cited**

U.S. PATENT DOCUMENTS

- 3,825,427 A 7/1974 Inoue et al.  
3,877,941 A 4/1975 Lohmann  
3,961,948 A 6/1976 Saeva  
4,425,161 A \* 1/1984 Shibahashi et al. ..... 106/31.17  
4,598,035 A 7/1986 Usami et al.  
4,659,649 A 4/1987 Dickinson et al.  
4,931,337 A \* 6/1990 Miyazaki et al. ..... 428/64.8  
5,124,236 A 6/1992 Yamaguchi et al.  
5,262,280 A 11/1993 Knudsen et al.  
5,376,511 A 12/1994 Tatezono et al.  
5,458,874 A 10/1995 Pereira et al.  
5,677,107 A 10/1997 Neckers  
5,691,100 A 11/1997 Kudo et al.  
5,691,395 A 11/1997 Knudsen et al.  
5,747,225 A 5/1998 Manico et al.  
6,067,185 A 5/2000 Albert et al.  
6,103,378 A 8/2000 Yao et al.  
6,200,646 B1 3/2001 Neckers et al.  
6,528,221 B2 3/2003 Takezawa et al.  
6,579,662 B1 6/2003 Zheng et al.  
6,680,281 B2 1/2004 Tajiri et al.  
6,761,758 B2 7/2004 Boils-Boissier et al.  
6,866,981 B2 3/2005 Furukawa et al.  
6,867,408 B1 3/2005 Gu et al.  
6,906,118 B2 6/2005 Goodbrand et al.  
7,018,714 B2 3/2006 Kobayashi et al.  
7,057,054 B2 6/2006 Irie  
7,205,088 B2 4/2007 Iftime et al.  
7,214,456 B2 5/2007 Iftime et al.  
7,229,740 B2 6/2007 Iftime et al.  
7,256,921 B2 \* 8/2007 Kumar et al. ..... 359/241  
7,332,257 B2 \* 2/2008 Miyako et al. ..... 430/270.1

- 7,381,506 B2 \* 6/2008 Iftime et al. ..... 430/19  
7,441,887 B2 \* 10/2008 Senga et al. ..... 347/107  
2002/0160318 A1 10/2002 Richter et al.  
2003/0130456 A1 7/2003 Kim et al.  
2005/0012998 A1 \* 1/2005 Kumar et al. ..... 359/494  
2005/0244744 A1 11/2005 Kazmaier et al.  
2005/0269556 A1 12/2005 Evans et al.  
2006/0001944 A1 1/2006 Chopra et al.  
2006/0222972 A1 10/2006 Chopra et al.  
2006/0222973 A1 10/2006 Iftime et al.  
2006/0236470 A1 10/2006 Sabnis et al.  
2006/0251988 A1 11/2006 Iftime et al.  
2006/0257785 A1 11/2006 Johnson  
2007/0054215 A1 3/2007 Iftime et al.  
2007/0072110 A1 3/2007 Iftime et al.  
2007/0112103 A1 5/2007 Zhou et al.

FOREIGN PATENT DOCUMENTS

- |    |              |         |
|----|--------------|---------|
| CA | 2 053 094 A1 | 4/1992  |
| DE | 29 06 193 A1 | 8/1980  |
| EP | 1 367 111    | 12/2003 |
| EP | 1 405 891    | 4/2004  |
| EP | 1 591 829    | 11/2005 |
| EP | 1 591 831    | 11/2005 |
| FR | 2774998      | 8/1999  |
| GB | 2 430 257    | 3/2007  |

(Continued)

OTHER PUBLICATIONS

Machine translation of JP 2005-255490.\*

U.S. Appl. No. 10/834,722, filed Apr. 29, 2004, Iftime et al.

U.S. Appl. No. 10/835,518, filed Apr. 29, 2004, Kazmaier et al.

U.S. Appl. No. 11/123,163, filed May 6, 2005, Iftime et al.

U.S. Appl. No. 11/220,572, filed Sep. 8, 2005, Iftime et al.

James T.C. Wojtyk et al., "Effects of metal ion complexation on the spiropyran-merocyanine interconversion:development of a thermally stable photo-switch," *J. Chem. Soc. Chem. Comm.*; pp. 1703-1704, 1998.

M. Irie, "Diarylethene for Memories and Switches," *Chem Reviews*, 100, pp. 1685-1716 (2000).

Kentaro Morimitsu et al., "Dithienylethenes With a Novel Photochromic Performance," *J. Org. Chem.*, vol. 67, pp. 4574-4578 (2002).

(Continued)

Primary Examiner—Amanda C. Walke

(74) Attorney, Agent, or Firm—Oliff & Berridge, PLC

(57) **ABSTRACT**

An image forming medium includes a substrate, and an imaging layer coated on or impregnated into the substrate, wherein the imaging layer includes an imaging composition including a photochromic or photochromic-thermochromic material and an infrared absorbent dissolved or dispersed in a solvent or polymeric binder; wherein the infrared absorber absorbs infrared light of a wavelength in a range from about 730 nm to about 1500 nm; and wherein the imaging composition is imageable by light of a first wavelength and erasable in a short time period by a combination of infrared radiation and light of a second wavelength and exhibits a reversible transition between a colorless and a colored state.

## FOREIGN PATENT DOCUMENTS

|    |                   |         |
|----|-------------------|---------|
| JP | 57-136645         | 8/1982  |
| JP | A-61-175087       | 8/1986  |
| JP | A-5-265129        | 10/1993 |
| JP | A-11-30835        | 2/1999  |
| JP | A 11-322739       | 11/1999 |
| JP | A 2000-256347     | 9/2000  |
| JP | A-2002-179672     | 6/2002  |
| JP | A-2002-240441     | 8/2002  |
| JP | A-2002-285146     | 10/2002 |
| JP | A-2003-255489     | 9/2003  |
| JP | A-2003-255490     | 9/2003  |
| JP | A-2004-039009     | 2/2004  |
| JP | A-2004-045037     | 2/2004  |
| JP | A-2004-091638     | 3/2004  |
| JP | A-2004-149501     | 5/2004  |
| JP | A-2004-256780     | 9/2004  |
| JP | A-2005-082507     | 3/2005  |
| JP | A-2005-250463     | 9/2005  |
| WO | WO 97/31033       | 8/1997  |
| WO | WO 00/16985 A1    | 3/2000  |
| WO | WO 2006/039130 A1 | 4/2006  |
| WO | WO 2007/105699 A1 | 9/2007  |
| WO | WO 2008/043853 A2 | 4/2008  |

## OTHER PUBLICATIONS

Kentaro Morimitsu et al., "Thermal Cycloreversion Reaction of a Photochromic Dithienylperfluorocyclopentene with *tert*-Butoxy Substituents at the Reactive Carbons," The Chemical Society of Japan, 2002, p. 572-573.

U.S. Appl. No. 11/762,152, filed Jun. 13, 2007, to Iftime et al.

U.S. Appl. No. 11/762,327, filed Jun. 13, 2007, to Iftime et al.

U.S. Appl. No. 11/762,147, filed Jun. 13, 2007, to Iftime et al.

U.S. Appl. No. 11/762,098, filed Jun. 13, 2007, to Iftime et al.

U.S. Appl. No. 11/762,157, filed Jun. 13, 2007, to Iftime et al.

U.S. Appl. No. 11/762,153, filed Jun. 13, 2007, to Iftime et al.

U.S. Appl. No. 11/762,144, filed Jun. 13, 2007, to Kazmaier et al.

U.S. Appl. No. 11/762,150, filed Jun. 13, 2007, to Norsten et al.

U.S. Appl. No. 11/762,107, filed Jun. 13, 2007, to Iftime et al.

U.S. Appl. No. 11/762,176, filed Jun. 13, 2007, to Norsten et al.

U.S. Appl. No. 11/762,307, filed Jun. 13, 2007, to Norsten et al.

U.S. Appl. No. 11/762,159, filed Jun. 13, 2007, to Kazmaier et al.

U.S. Appl. No. 11/762,311, filed Jun. 13, 2007, to Kazmaier et al.

U.S. Appl. No. 11/762,177, filed Jun. 13, 2007, to Norsten et al.

Wojtyk et al., "Effects of metal ion complexation on the spiropyran-merocyanine interconversion: development of a thermally stable photo-switch," J. Chem. Soc. Chem. Comm., pp. 1703-1704, 1998.

"Dolch Introduces World's First Ruggedized Notebook with Integrated Printer" available at <http://news.thomasnet.com/fullstory/7005/447>, pp. 1-4, Feb. 6, 2002.

Masamitsu Shirai et al., "Photoacid and Photobase Generators: Chemistry and Applications to Polymeric Materials," *Prog. Polym. Sci.* vol. 21, pp. 1-45 (1996).

T. Hirose et al., "Self-Assembly of Photochromic Diarylethenes With Amphiphilic Side Chains: Reversible Thermal and Photochemical Control," *J. Org. Chem.*, 71, pp. 7499-7508 (2006).

T. Norsten et al., "Photoregulation of Fluorescence in a Porphyrinic Dithienylethene Photochrome," *J. Am. Chem. Soc.*, 123(8), pp. 1784-1785 (2001).

Vladimir I. Minkin, "Photo-, Thermo-, Solvato-, and Electrochromic Spiroheterocyclic Compounds," *Chemical Reviews*, 104, 5, pp. 2751-2776 (2004).

Takayuki Suzuki et al., "Stabilization of the merocyanine form of photochromic compounds in fluoro alcohols is due to a hydrogen bond", *Chem. Commun.*, 2685-2686 (1998).

Ronald F.M. Lange et al., "Supramolecular polymer interactions based on the alternating copolymer of styrene and Maleimide" *Macromolecules*, 28, 782-783 (1995).

Vladimir I. Minkin et al., "Perimidine spirocyclohexa dienones" in *Organic Photochromic and Thermochromic Compounds*, V1, Plenum Press, pp. 315-340 (1999).

John Biteau et al., "Photochromism of Spirooxazine-Doped Gels," *J. Phys. Chem.*, 100, 9024-9031(1996).

Leonard J. Prins et al., "Noncovalent Synthesis Using Hydrogen Bonding," *Angew. Chem. Int. Ed.*, 40, 2382-2426 (2001).

Terry M. Cresp et al., "A Synthesis of  $\alpha\beta$ -Unsaturated Aldehydes," *J. Chem. Soc., Perkin Trans.*, 1, pp. 37-41 (1974).

Elliot Berman et al., "Photochromic Spiropyrans. I. The Effect of Substituents on the Rate of Ring Closure," *J. Am. Chem. Soc.*, 81, 5605-5608 (1959).

Sheng-Hua Liu et al., "Synthesis of Negative Photochromic Crowned Spiropyropyrans," *Syn. Commun.*, 30, 5, 895-902 (2000).

Yu M. Chunaev et al., "Reaction of the Fischer Base With Nitro- and Bromo-Substituted  $\alpha$ -Hydroxycinnamaldehydes," *Chem. Heterocycl. Compd.*, 628-631 (1984).

O.M. Babeshko et al., "Spiro-2H-Oxocines", *Khimiya Geterotsiklicheskikh Soedinenii*, No. 11, pp. 1490-1492, Nov. 1976.

Samir Kumar Mandal et al., "Titanocene(III) mediated radical cyclizations of epoxides for the synthesis of medium-sized cyclic ethers", *Tetrahedron*, vol. 63, pp. 11341-11348, 2007.

Sep. 9, 2009 European Office Action issued in European Application No. 08 155 983.3 - 1217.

\* cited by examiner

INKLESS REIMAGEABLE PRINTING PAPER  
AND METHOD

## TECHNICAL FIELD

This disclosure is generally directed to a substrate, method, and apparatus for inkless printing on reimageable paper. More particularly, in embodiments, this disclosure is directed to an inkless reimageable printing substrate, such as inkless printing paper utilizing a composition that is imageable by light and erasable in a short time period by a combination of light and infrared radiation, where the composition includes an infrared absorber such as infrared dye and exhibits a reversible transition between a colorless and a colored state. Imaging is conducted, for example, by applying UV light to cause a color change, and erasing is conducted by applying a combination of visible light and infrared radiation to the imaging material to reverse the color change. Other embodiments are directed to inkless printing methods using the inkless printing substrates, and apparatus and systems for such printing.

CROSS-REFERENCE TO RELATED  
APPLICATIONS

Disclosed in commonly assigned U.S. patent application Ser. No. 11/762,177, filed Jun. 13, 2007, is a photochromic material represented by the general formula (I)



wherein:

each X independently represents hydrogen, an allyl chain having 1 to 20 carbon atoms, bromine, chlorine or an iodine atom,

A represents a group of formula (a)-(c), and

B represents a group of formula (d)-(f),



-continued



[d]

[e]

[f]

wherein:

R<sub>4</sub> represents an aryloxy group, a substituted and unsubstituted heteroaromatic group, an alkoxy group, or a substituted alkoxy group, where the alkyl portion of the alkoxy group represents a straight, branched or cyclic, substituted or unsubstituted, alkyl group of from 1 to about 40 carbon atoms,

R<sub>5</sub> represents an aryl group, a substituted or unsubstituted alkylaryl group wherein hetero atoms either may or may not be present in the alkyl portion of the alkylaryl group or the aryl portion of the alkylaryl group, a cyano group, a carboxylic acid group, or an unsaturated alkene group,

R<sub>6</sub> represents a hydrogen atom, an alkyl group, a halogen atom, an alkoxy group, a fluoroalkyl group, a cyano group, an aryl group, or a substituted alkylaryl group,

R<sub>7</sub> represents an alkyl group, an aryl group, an alkylaryl group including substituted alkylaryl groups, unsubstituted alkylaryl groups, and wherein hetero atoms either may or may not be present in the alkyl portion of the alkylaryl group or the aryl portion of the alkylaryl,

R<sub>8</sub> represents an aryloxy group, substituted and unsubstituted heteroaromatic group, or an alkoxy group or substituted alkoxy group where the alkyl portion of the alkoxy group represents a straight, branched or cyclic, substituted or unsubstituted, alkyl group of from 1 to about 40 carbon atoms,

R<sub>9</sub> represents an aryl group, a substituted or unsubstituted alkylaryl groups wherein hetero atoms either may or may not be present in the alkyl portion of the alkylaryl group or the aryl portion of the alkylaryl group, a cyano group, a carboxylic acid group, or an unsaturated alkene group,

R<sub>10</sub> represents a hydrogen atom, an alkyl group, a halogen atom, an alkoxy group, a fluoroalkyl group, a cyano group, an aryl group, or a substituted alkylaryl group,

R<sub>11</sub> represents an alkyl group, an aryl group, or a substituted or unsubstituted alkylaryl group wherein hetero atoms either may or may not be present in the alkyl portion of the alkylaryl group or the aryl portion of the alkylaryl, and

U and Z each independently represent sulfur or oxygen atoms. Also disclosed is an image forming medium, comprising a paper substrate; and an imaging layer coated on or impregnated into said paper substrate, wherein the imaging layer comprises an imaging composition comprising the

above photochromic material dissolved or dispersed in a solvent or polymeric binder; wherein the imaging composition exhibits a reversible transition between a colorless and a colored state.

Disclosed in commonly assigned U.S. patent application Ser. No. 11/762,159, filed Jun. 13, 2007, is an image forming medium, comprising a substrate; and an imaging layer coated on or impregnated into said substrate, wherein the imaging layer comprises an imaging composition comprising a photochromic or photochromic-thermochromic material dissolved or dispersed in a solvent or polymeric binder; wherein the imaging composition is imageable by light of a first wavelength and erasable in a short time period by a combination of heat and light of a second wavelength such that simultaneous erase with heat and light of the second wavelength is faster than erase by heat alone and exhibits a reversible transition between a colorless and a colored state.

The entire disclosure of the above-mentioned applications are totally incorporated herein by reference.

#### BACKGROUND

Inkjet printing is a well-established market and process, where images are formed by ejecting droplets of ink in an image-wise manner onto a substrate. Inkjet printers are widely used in home and business environments, and particularly in home environments due to the low cost of the inkjet printers. The inkjet printers generally allow for producing high quality images, ranging from black-and-white text to photographic images, on a wide range of substrates such as standard office paper, transparencies, and photographic paper.

However, despite the low printer costs, the cost of replacement inkjet cartridges can be high, and sometimes higher than the cost of the printer itself. These cartridges must be replaced frequently, and thus replacement costs of the ink cartridges is a primary consumer complaint relating to inkjet printing. Reducing ink cartridge replacement costs would thus be a significant enhancement to inkjet printing users.

In addition, many paper documents are promptly discarded after being read. Although paper is inexpensive, the quantity of discarded paper documents is enormous and the disposal of these discarded paper documents raises significant cost and environmental issues. Accordingly, there is a continuing desire for providing a new medium for containing the desired image, and methods for preparing and using such a medium. In aspects thereof it would be desirable to be reusable, to abate the cost and environmental issues, and desirably also is flexible and paper-like to provide a medium that is customarily acceptable to end-users and easy to use and store.

Although there are available technologies for transient image formation and storage, they generally provide less than desirable results for most applications as a paper substitute. For example, alternative technologies include liquid crystal displays, electrophoretics, and gyricon image media. However, these alternative technologies may not in a number of instances provide a document that has the appearance and feel of traditional paper, while providing the desired reimageability.

Imaging techniques employing photochromic materials, that is materials which undergo reversible or irreversible photoinduced color changes are known, for example, U.S. Pat. No. 3,961,948 discloses an imaging method based upon visible light induced changes in a photochromic imaging layer containing a dispersion of at least one photochromic material in an organic film forming binder.

These and other photochromic (or reimageable or electric) papers are desirable because they can provide imaging media that can be reused many times, to transiently store images and documents. For example, applications for photochromic based media include reimageable documents such as, for example, electronic paper documents. Reimageable documents allow information to be kept for as long as the user wants, then the information can be erased or the reimageable document can be re-imaged using an imaging system with different information.

Although the above-described approaches have provided reimageable transient documents, there is a desire for reimageable paper designs that provide longer image life-times, and more desirable paper-like appearance and feel.

A problem associated with transient documents is balancing the demands of image stability to ambient conditions, and ability to quickly erase and reimage the document when desired. For example, while some materials such as alkoxy dithienylethenes show room temperature image stability for weeks and very slow light induced fading under ambient conditions, image erasure in visible light or under thermal heating is slow and occurs at too high a heating temperature. It is possible to reduce the erase time by using bulky substituents, but this kind of structural change may also increase the fading rate at ambient temperature and reduce the archival life of the image. It is important to modify the erase conditions in such a way that faster erase times are achieved while maintaining long (such as more than 3 days) image lifetime. A solution is dual input erase, using simultaneous heating and VIS light exposure of the colored state, as disclosed in U.S. patent application Ser. No. 11/762,159, filed Jun. 13, 2007. A dual erase system requires such a design that a heating element is in very close proximity to an erasing light source. Since they can not be in perfect contact, heat energy is lost, reducing the erase efficiency.

Many available visible light sources required for the erase step also have a significant IR light component. This IR radiant energy is converted into heat upon absorption by the substrate. However, with erasable papers in the prior art, much of this IR energy is practically wasted because it is poorly absorbed by the media.

Faster erasing time and more practical erasing conditions are important in order to make reimageable paper documents practical for commercial use. This can be achieved if the IR energy is efficiently captured in order to heat the photochromic material.

#### SUMMARY

It is desirable for some uses that an image formed on a reimageable medium such as a transient document remains stable for extended time periods, without the image or image contrast being degraded by exposure to ambient UV light or having the image self-erase too quickly because of ambient thermal energy. However, it is also desired that the image can be erased in a short time period when desired, to permit reimaging of the medium. Reimageable paper documents should maintain a written image for as long as the user needs to view it, without the image being degraded by ambient light or prematurely by ambient heat. The image may then be erased or replaced with a different image by the user on command, with the erasing being conducted in a short time period.

The present disclosure addresses these and other needs, in embodiments, by providing a reimageable image forming medium utilizing a composition that is imageable by light and eraseable in a short time period by a combination light and

infrared radiation, where the composition includes an infrared absorber such as an infrared dye and exhibits a reversible transition between a colorless and a colored state. Imaging is conducted by applying, for example, UV light to the imaging material to cause a color change, and erasing is conducted by applying, for example, a combination of light and infrared radiation to the imaging material to reverse the color change. The present disclosure in other embodiments provides an inkless printing method using the reimageable inkless printing substrates, and apparatus and systems for such printing.

The present disclosure thereby provides a printing media, method, and printer system for printing images without using ink or toner. The paper media has a special imageable composition that is printed with light, can remain in the printed form for an extended period of time, such as more than three days, more than one week, or more than one month, and can be erased with light and infrared radiation in a short time period. The paper media thus allows image formation and erasure using a printer that does not require ink or toner replacement, and instead images the paper using a UV light source, such as a LED. The compositions and methods of the present disclosure also provide transient images that last for significantly longer periods of time, while still being able to be erased in a short period of time. These advantages, and others, allow wider application of the reimageable transient documents.

The present disclosure describes special reimageable compositions including a photochromic or photochromic-thermochromic material and an infrared absorber such as an infrared dye, where erasing simultaneously with visible light and infrared radiation provides faster erase than erasing with heat or visible light alone. When the infrared absorber is absent, the IR radiation emitted by the light source is only partially used, essentially producing heat due to absorption by the substrate (such as paper) or of the polymer binder, which indirectly heats the photochromic molecules. However, when the infrared absorber is present in the photochromic composition, it captures the otherwise wasted or inefficiently used IR radiation and converts it into heat that is used by the neighboring photochromic molecules producing faster erase when compared to the situation when the infrared absorber is absent.

In an embodiment, the present disclosure provides an image forming medium, comprising

a substrate; and

an imaging layer coated on or impregnated into said substrate, wherein the imaging layer comprises an imaging composition comprising a photochromic or photochromic-thermochromic material and an infrared absorber dissolved or dispersed in a solvent or polymeric binder;

wherein the infrared absorber absorbs infrared light of a wavelength in a range from about 730 nm to about 1500 nm; and

wherein the imaging composition is imageable by light of a first wavelength and erasable in a short time period by a combination of infrared radiation and light of a second wavelength and exhibits a reversible transition between a colorless and a colored state.

In another embodiment, the present disclosure provides a system for imaging such an image forming medium, the system comprising:

a printer comprising an imaging member that outputs the first wavelength and an erase component that outputs infrared radiation and the second wavelength, that is capable of heating and flooding the image forming medium with heat and light of the second wavelength simultaneously.

## DETAILED DESCRIPTION OF EXEMPLARY EMBODIMENTS

Generally, in various exemplary embodiments, there is provided an inkless reimageable paper or image forming medium formed using a composition that is imageable by light and erasable in a short time period by a combination of light and infrared radiation, such as comprising an infrared absorber such as an infrared dye and a photochromic material dispersed in a solvent or polymeric binder, where the composition exhibits a reversible transition between a colorless and a colored state. Exposing the imaging layer to a first stimulus such as UV light irradiation causes the photochromic material to convert from the colorless state to a colored state. Likewise, exposing the imaging layer to a second stimulus such as a combination of visible light irradiation and infrared radiation, whereby the infrared absorber absorbs the infrared radiation and locally heats the imaging layer, causes the photochromic material to convert from the colored state to the colorless state. By a colored state, in embodiments, refers to for example, the presence or absorption of visible wavelengths; likewise, by a colorless state, in embodiments, refers to for example, the complete or substantial absence of visible wavelengths or the complete or substantial absence of absorption in the visible region of the spectrum (400-800 nanometers).

In the prior art, a trade-off has been between imaging duration, and energy required for image erase. Many photochromic compounds that require low levels of energy for erasing, have a short image lifetime, while other photochromic compounds that have a longer image lifetime, require higher levels of energy for erasing. For example, images formed from some photochromic compounds can be acceptably erased using strong visible light and heating to 160° C. within about 10 second, but the image has a duration of only about three days, which is too short for many applications. On the other hand, images formed from other photochromic compounds can acceptably have an image duration of one month or more, but the images can only be erased using strong visible light and heating to 160° C. in periods of time of two minutes or more, which is too long for many applications. Embodiments of this disclosure address these problems by using the long image duration compounds, but remedying the long erase time by incorporating infrared absorbers into the composition that absorb infrared radiation in the erasing cycle to speed the erase process.

Erasing of a photochromic reimageable paper can be accomplished by light or heat alone. However, paper is a fragile substrate and one cannot increase the thermal input to high values without damaging or wrinkling the paper substrate. Furthermore, erase of a photochromic material using heat is a typical chemical process and has an energy barrier that can be described by the Arrhenius equation. One form of the equation is  $k = A * \exp[-E_a / (R * T)]$  where  $E_a$  is the activation energy. Erase of the image can be accomplished at lower temperature or more rapidly at the same temperature by adjusting the substituents so that  $E_a$  is reduced. However this modification will necessarily also increase the rate of fading at ambient temperature, perhaps to an unacceptable rate. Further, often the heat that can be applied to the substrate is desirably applied using an infrared radiation source; however, paper substrates and the like do not efficiently absorb infrared radiation efficiently at a rate that would provide desirable erasing. The dual erase method of embodiments overcomes this deficiency because the infrared absorber more efficiently absorbs the infrared radiation and converts it to heat at the

image location, to provide faster erasing rates. The image can thus be erased in a short time period.

As used herein, "short time period" refers, for example, to the erasing being conducted such that the absorbance of the imaging composition in the visible light range at the maximum absorption, such as about 640 nm, is reduced to one half of its initial value within a time period of about 10 minutes or less upon exposure to a light source emitting simultaneously visible and IR light such as a quartz halogen incandescent heat lamp, which can provide both visible light and IR light. For example, in some embodiments, the erasing can be conducted such that the absorbance of the imaging composition at about 640 nm is reduced from an absorbance of 0.7 to 0.35 within a time period of about 10 minutes or less upon exposure to a light source emitting simultaneously visible and IR light, while in other embodiments the erasing can be conducted such that the absorbance of the imaging composition at about 640 nm is reduced to one half of its initial value within a time period of about 5 minutes or less than about 2 minutes or less than about 1 minute. Commonly available usable light sources include quartz lamps, with a tungsten filament, quartz tubes, LED bars, xenon flash light sources, and the like.

Photochromism and thermochromism are defined as the reversible photocoloration of a molecule from exposure to light (electromagnetic radiation) and heat (thermal radiation) based stimuli respectively. Typically photochromic molecules undergo structural and/or electronic rearrangements when irradiated with UV light that converts them to a more conjugated colored state. In the case of photochromic molecules, the colored state can typically be converted back to their original colorless state by irradiating them with visible light. In some cases thermal energy can also be used to decolorize a photochrome. Dithienylethenes and fulgides are examples of purely photochromic molecules. If the interconversion is also capable thermally (by applying heat), as is the case in alkoxy substituted dithienylethenes, spiropyrans, azabenzenes, schiff bases and the like, the molecules are classified as both thermochromic and photochromic. Photochromic compounds are completely bi-stable in absence of light whereas photochromic-thermochromic hybrid compounds will fade in the absence of light through a thermal process to the thermodynamically more stable colorless state. To create a stable reimageable document it is desired to stabilize the colored state, specifically to ambient conditions that the document will encounter in everyday life, such as broad band light and various heating/cooling conditions. However, it is also desirable that the compounds be capable of reversion back to the colorless state in a short time period, when erasing is desired.

In embodiments, the image forming medium generally comprises an imaging layer coated on or impregnated in a suitable substrate material, or sandwiched or laminated between a first and a second substrate material (i.e., a substrate material and an overcoat layer). The imaging layer comprises an infrared absorber such as an infrared dye and a photochromic or photochromic-thermochromic material dispersed in a solvent or polymeric binder. The imaging composition is imageable by light and eraseable in a short time period by a combination of light and infrared radiation, and exhibits a reversible transition between a colorless and a colored state.

The imaging layer can include any suitable infrared absorber, photochromic material and solvent or polymer binder. For example, the photochromic material and solvent or polymer binder are selected such that when the photochromo-

mic material is dissolved or dispersed in the solvent or polymer binder, the photochromic material is in its clear state. However, when the photochromic material is exposed to a first stimulus, such as ultraviolet light, the photochromic material isomerizes to a more polar colored form. This color change can be reversed, and thus the image "erased" and the photochromic paper returned to a blank state. In the colored state, the image can remain visible for a period of two days or more, such as a week or more or one month or more, providing increased usefulness of the photochromic paper, but can be readily erased in a short time period when desired.

In embodiments, the photochromic material is a photochromic-thermochromic hybrid compound that can be imaged by UV light alone and that can be erased using a combination of visible light and heat created by the absorption of infrared radiation by an infrared absorber. This erasing in the presence of visible light and heat with an infrared absorber represents a significant decrease in the erase time, as compared to erasing by light and/or heat alone.

The photochromic material is dispersed in a solvent or polymeric binder, where the photochromic material exhibits a reversible transition between a colorless and a colored state. The photochromic material exhibits photochromism and thermochromism, thus exhibiting a reversible transformation induced in one or both directions by absorption of an electromagnetic radiation and heat, between two forms having different absorption spectra. The first form is thermodynamically stable and may be induced by absorption of light such as ultraviolet light to convert to a second form. The reverse reaction from the second form to the first form may occur, for example, thermally and by absorption of light such as visible light. Various exemplary embodiments of the photochromic material may also encompass the reversible transformation of the chemical species among three or more forms in the event it is possible that reversible transformation occurs among more than two forms. The photochromic material of embodiments may be composed of one, two, three, four, or more different types of photochromic materials, each of which has reversibly interconvertible forms. As used herein, the term "photochromic material" refers to all molecules of a specific species of the photochromic material, regardless of their temporary isomeric forms. In various exemplary embodiments, for each type of photochromic material, one form may be colorless or weakly colored and the other form may be differently colored.

In embodiments, the reimageable paper also generally comprises a solvent or polymer binder mixture of an infrared absorber and a photochromic material dispersed or dissolved in the solvent or polymer binder, with the mixture coated on a suitable substrate material, or sandwiched between a first and a second substrate material. If desired, the mixture can be further constrained on the substrate material, or between the first and second substrate materials, such as by microencapsulating the solvent mixture, or the like.

In particular embodiments, the photochromic material is selected from any class of photochromic materials, including but not limited to spiropyrans, dithienylethenes, naphthopyrans or chromenes and fulgides.

Accordingly, the substituted diarylethene suitable for use in embodiments are those that can be represented by the following general formulas [I]-[VII]:



In formula [I], X independently represents H; a halogen such as chlorine, fluorine, bromine, or the like; a straight or branched, substituted or unsubstituted, allyl group of from 1 to about 20 or to about 40 carbon atoms, such as methyl, ethyl, propyl, butyl, or the like, where the substitutions can include halogen atoms, hetero atoms (such as oxygen groups, nitrogen groups, and the like), and the like.



In formula [II], X represents S or O.



In formula [IV], X represents S, O or C=O, Y represents O, 45 CH<sub>2</sub> or C=O.



In formula [V], Y represents CH<sub>2</sub> or C=O.



In formula [VI], X represents CH or N.



In formula [VII], Y represents CH<sub>2</sub> or C=O.

10 In the general formulas [I]-[VII], R<sub>1</sub>, R<sub>2</sub> are each independently selected from an alkyl group, including substituted allyl groups, unsubstituted alkyl groups, linear alkyl groups, and branched alkyl groups, and wherein hetero atoms such as oxygen, nitrogen, sulfur, silicon, phosphorus, boron, and the like either may or may not be present in the alkyl group, a halogen group, an alkoxy group, a cyano group, a nitro group, an amino group, an amide group, an aryl group, an alkylaryl group, including substituted alkylaryl groups, unsubstituted alkylaryl groups, and wherein hetero atoms either may or may

15 not be present in the alkyl portion of the alkylaryl group or the aryl portion of the alkylaryl group, R<sub>3</sub> represents an allyl group, including substituted alkyl groups, unsubstituted alkyl groups, linear allyl groups, and branched allyl groups, and wherein hetero atoms such as oxygen, nitrogen, sulfur, silicon, phosphorus, boron, and the like either may or may not be present in the alkyl group, A represents substituents [a] or [b] or [c], and B represents substituents [d] or [e] or [f] shown below,



In substituents [a]-[c], R<sub>4</sub> represents an aryloxy group including phenyl, naphthyl and the like and substituted and

11

unsubstituted heteroaromatic group, an alkoxy group or substituted alkoxy group where the alkyl portion of the alkoxy group represents a straight, branched or cyclic, substituted or unsubstituted, alkyl group of from 1 to about 20 or about 40 carbon atoms, such as methyl, ethyl, propyl, butyl, isopropyl, cyclohexyl, isoborneol or the like, where the substitutions can include halogen atoms, hetero atoms (such as oxygen groups, nitrogen groups, and the like), and the like, R<sub>5</sub> represents an aryl group, or an alkylaryl group including substituted alkylaryl groups, unsubstituted alkylaryl groups, and wherein hetero atoms either may or may not be present in the alkyl portion of the alkylaryl group or the aryl portion of the alkylaryl, a cyano group, a carboxylic acid group or an unsaturated alkene group, R<sub>6</sub> represents a hydrogen atom, an allyl group, a halogen atom, and alkoxy group, a fluoroalkyl group, a cyano group, an aryl group, or a substituted alkylaryl group, R<sub>7</sub> represents an alkyl group and aryl group, or an alkylaryl group including substituted alkylaryl groups, unsubstituted alkylaryl groups, and wherein hetero atoms either may or may not be present in the allyl portion of the alkylaryl group or the aryl portion of the alkylaryl and U represents O or S.

In substituents [d]-[f], R<sub>8</sub> represents an aryloxy group including phenyl, naphthyl and the like, and substituted and unsubstituted heteroaromatic group, or an alkoxy group or substituted alkoxy group where the alkyl portion of the alkoxy group represents a straight, branched or cyclic, substituted or unsubstituted, allyl group of from 1 to about 20 or about 40 carbon atoms, such as methyl, ethyl, propyl, butyl, isopropyl, cyclohexyl, isoborneol or the like, where the substitutions can include halogen atoms, hetero atoms (such as oxygen groups, nitrogen groups, and the like), and the like, R<sub>9</sub> represents an aryl group, or an alkylaryl group including substituted alkylaryl groups, unsubstituted alkylaryl groups, and wherein hetero atoms either may or may not be present in the alkyl portion of the alkylaryl group or the aryl portion of the alkylaryl, a cyano group, a carboxylic acid group or an unsaturated alkene group, R<sub>10</sub> represents a hydrogen atom, an alkyl group, a halogen atom, and alkoxy group, a fluoroalkyl group, a cyano group, an aryl group, or a substituted alkylaryl group, R represents an alkyl group and aryl group, or an alkylaryl group including substituted alkylaryl groups, unsubstituted alkylaryl groups, and wherein hetero atoms either may or may not be present in the alkyl portion of the alkylaryl group or the aryl portion of the alkylaryl and Z represents O or S.

In certain embodiments, the substituted diarylethenes of formulas [I]-[VII] are those compounds where R<sub>4</sub> and R<sub>8</sub> are the same alkoxy containing substituents. In this case it is necessary for the alkyl or substituted allyl groups to contain 4 or more carbon atoms. This is a requirement for adequate thermal-based cycloreversion reaction times for the present applications. In other embodiments, however, the alkoxy substituents of R<sub>4</sub> and R<sub>8</sub> can be different alkoxy substituents. In this case as well, it is preferred that either at least one or both of the alkoxy groups contain 4 or more carbon atoms.

One example class, the alkoxy diethienylethenes are shown below, but many other classes will be evident to someone skilled in the art. The alkoxy substituted dithienylethene suitable for use in embodiments are those that can be represented by the following reversible transition:

12



where each R, which can be the same or different, represents a straight or branched alkyl group such as methyl, ethyl, propyl, i-propyl, butyl, and the like, or cyclic alkyl group such as cyclopropyl, cyclohexyl, and the like, and including unsaturated alkyl groups, such as vinyl (H<sub>2</sub>C=CH—), allyl (H<sub>2</sub>C=CH—CH<sub>2</sub>—), propynyl (HC≡C—CH<sub>2</sub>—), and the like, where for each of the foregoing, the alkyl group has from 1 to about 20, such as from 1 to about 15, 1 to about 10, or 1 to about 6 or to about 8, carbon atoms. Each R independently can also be aryl, including phenyl, naphthyl, phenanthrene, anthracene, substituted groups thereof, and the like, and having from about 6 to about 30 carbon atoms such as from about 6 to about 20 carbon atoms; arylalkyl; such as having from about 7 to about 50 carbon atoms such as from about 7 to about 30 carbon atoms; silyl groups; nitro groups; cyano groups; halide atoms, such as fluoride, chloride, bromide, iodide, and astatide; amine groups, including primary, secondary, and tertiary amines; hydroxy groups; alkoxy groups, such as having from 1 to about 50 carbon atoms such as from 1 to about 30 carbon atoms; aryloxy groups, such as having from about 6 to about 20 carbon atoms; alkylthio groups, such as having from 1 to about 50 carbon atoms such as from 1 to about 30 carbon atoms; arylthio groups, such as having from about 6 to about 30 carbon atoms such as from about 6 to about 20 carbon atoms; aldehyde groups; ketone groups; ester groups; amide groups; carboxylic acid groups; sulfonic acid groups; and the like. The group can be unsubstituted or substituted, for example, by silyl groups; nitro groups; cyano groups; halide atoms, such as fluoride, chloride, bromide, iodide, and astatide; amine groups, including primary, secondary, and tertiary amines; hydroxy groups; alkoxy groups, such as having from 1 to about 20 carbon atoms such as from 1 to about 10 carbon atoms; aryloxy groups, such as having from about 6 to about 20 carbon atoms such as from about 6 to about 10 carbon atoms; alkylthio groups, such as having from 1 to about 20 carbon atoms such as from 1 to about 10 carbon atoms; arylthio groups, such as having from about 6 to about 20 carbon atoms such as from about 6 to about 10 carbon atoms; aldehyde groups; ketone groups; ester groups; amide groups; carboxylic acid groups; sulfonic acid groups; and the

13

like. Specific examples of such compounds include those where R is methyl, ethyl, i-propyl, or cyclohexyl groups.

The alkoxy substituted dithienylethenes are more stable in their colored states than other substituted dithienylethenes, such as alkyl substituted dithienylethenes, to ambient visible light for longer periods of time. At the same time, the alkoxy substitution lowers the barrier to thermal de-colorization, or the reverse isomerization from the colored state back to the colorless state.

A particular advantage of the alkoxy modified dithienylethenes is that suitable selection of the alkoxy substituent can allow for specific tuning of the barrier to thermal erase. For example, thermal fading curves for different alkoxy modified dithienylethenes show, for example, that the barrier to thermal erasing can be tuned to be rapid and complete at elevated temperatures (such as about 100 to about 160° C.) while maintaining long-term thermal-based color stability at ambient temperatures (such as about 25 to about 70° C.) based on the structure of the alkoxy R-group substituent. Based on such thermal analysis, the half-life thermal stability of the specific compounds can be predicted to range from 2.2 years at 30° C. for the least thermally stable tert-butyl compound (see *Chem. Lett.* 2002, 572.), to 420 years at 30° C. for the methoxy compound.

The infrared absorber contained in the reimageable paper can be any suitable infrared absorber that can absorb energy in the infrared or near infrared range, and convert that energy to heat to heat the imaging composition to assist in conversion of the photochromic material from its colored state to its colorless state. The presence of the infrared absorber increases the absorption of IR radiation, because it absorbs also the IR energy that is not absorbed by the paper substrate. This results in faster localized heating of the photochromic molecules. Overall the photochromic material is thereby heated faster and to a higher temperature without increasing the energy consumption in the erasing step. As a result, faster erasing is achieved. This allows photochromic materials to be used providing longer image lifetime without the disadvantage of slow erasing.

Suitable infrared absorbers include, for example, infrared dyes. Suitable IR dyes generally have strong absorption of radiation in a range from about 730 nm to about 3 microns, preferably from about 730 nm to about 1.5 microns. This region of the spectrum is known as Near Infrared (NIR). Most of the commonly available substrates or polymeric binders have poor absorption of radiations having a corresponding wavelength smaller than 1.5 microns. Infrared absorbers thus compensate for the absorptions at wavelengths where the substrate or polymer binder do not absorb. Examples of suitable infrared absorbing dyes include for example diimmonium compounds, such as an aminium-salt-based compound described by the following formula (1) and/or a diimmonium-salt-based compound described by the following formula (2):

(1)



14

-continued

(2)



10 In the formulas (1) and (2) above, R<sub>1</sub> through R<sub>4</sub> each independently denote hydrogen atom, alkyl group, substitution allyl group, cyclic alkyl group, alkenyl group, alkyl group or substituted alkyl group, and X<sup>-</sup> denotes a suitable negative ion. The aminium-salt-based compound and the diimmonium-salt-based compound have a high infrared absorption and a light color that does not or does not significantly affect the hue of the imaging composition. For example, compounds CIR-960, CIR-961, CIR-963, CIR-1080, CIR-1081 and CIR-1083 manufactured by Nihon Karlit Company of Japan may be used for the infrared absorbed, in embodiments. Japan Carlit Co sells CIR108x and CIR96x NIR absorbing materials, with very little absorption in the VIS region of the spectrum, but with extremely strong absorption in the NIR, and H.W. Sands Corp. sells a whole range of NIR absorbing materials with fine tuned ranges of absorption in the NIR (from 650 nm to over 1000 nm), all of which can also be used in embodiments.

30 Other suitable infrared absorbers include, for example, indocyanine green, which is commercially available from Akorn, Inc. (Buffalo Grove, Ill.), under the name IC-GREEN<sup>TM</sup>, fluorescein isothiocyanate, rhodamine, phycoerythrin, phycocyanin, allophycocyanin, o-phthaldehyde, fluorescamine, Rose Bengal, trypan blue, and fluoro-gold. Dye analogs of the above infrared and near infrared dyes can 35 also be used, where a "dye analog" is a dye that has been chemically modified, but still retains its ability to fluoresce when exposed to radiant energy of an appropriate wavelength. In addition to the dyes mentioned, carbon nanoparticles could also be used in low percentages as IR absorbers to 40 enhance the IR absorption characteristics of the media.

Still other suitable infrared absorbers are described in, for example, U.S. Pat. Nos. 6,528,221 and 7,018,714, and in "Infrared Absorbing Dyes", Matsuoka, Masaru, ed., Plenum Press (1990) and "Near-Infrared Dyes for High Technology Applications", Daehne, S.; Resch-Genger, U.; Wolfbeis, O., Ed., Kluwer Academic Publishers, the entire disclosures of which are incorporated herein by reference.

50 Accordingly, in embodiments, the photochromic material can be readily converted from its colored state to its colorless state by exposure to suitable irradiation, such as a combination of visible light and infrared radiation. By "readily converted" herein is meant that the photochromic material can be converted from its colored state to its colorless state in a short 55 time period, as described above. In contrast, the photochromic material is not readily converted from its colored state to its colorless state in a short time period, that is, the absorbance of the imaging composition in the visible light range, such as about 640 nm, is not reduced from its initial absorbance to one half its value within a time period of about 10 minutes or less, 60 upon exposure visible light alone.

65 The infrared radiation used in activating the conversion can be any suitable radiation source, such as a IR lamp, near IR lamp, or the like. Typically used are quartz halogen incandescent heat lamps. Similarly, the visible light source used in activating the conversion can be any suitable light wavelength, for example from visible to ultraviolet, where visible

light is used in embodiments. The lighting can be provided by any suitable means, and can be of a narrow wavelength range or broad wavelength range. In an embodiment, a light source that provides both visible light wavelengths and infrared wavelength to provide heat can be used.

In one embodiment, the image forming material (photochromic material and infrared absorber) is dissolved or dispersed in any suitable carrier, such as a solvent, a polymer binder, or the like. Suitable solvents include, for example, straight chain aliphatic hydrocarbons, branched chain aliphatic hydrocarbons, and the like, such as where the straight or branched chain aliphatic hydrocarbons have from about 1 to about 30 carbon atoms. For example, a non-polar liquid of the ISOPARTM series (manufactured by the Exxon Corporation) may be used as the solvent. These hydrocarbon liquids are considered narrow portions of isoparaffinic hydrocarbon fractions. Other suitable solvent materials include, for example, the NORPARTM series of liquids, which are compositions of n-paraffins available from Exxon Corporation, the SOLTROLTM series of liquids available from the Phillips Petroleum Company, and the SHELLSOLTM series of liquids available from the Shell Oil Company. Mixtures of one or more solvents, i.e., a solvent system, can also be used, if desired. In addition, more polar solvents can also be used, if desired. Examples of more polar solvents that may be used include halogenated and nonhalogenated solvents, such as tetrahydrofuran, trichloro- and tetrachloroethane, dichloromethane, chloroform, monochlorobenzene, toluene, xylenes, acetone, methanol, ethanol, xylenes, benzene, ethyl acetate, dimethylformamide, cyclohexanone, N-methyl acetamide and the like. The solvent may be composed of one, two, three or more different solvents. When two or more different solvents are present, each solvent may be present in an equal or unequal amount by weight ranging for example from about 5% to 90%, particularly from about 30% to about 50%, based on the weight of all solvents.

Both compositions dispersable in either organic polymers or waterborne polymers can be used, depending on the used components. For example, for waterborne compositions, polyvinylalcohol is a suitable application solvent, and polymethylmethacrylate is suitable for organic soluble compositions.

Suitable examples of polymer binders include, but are not limited to, polyallylacrlylates like polymethyl methacrylate (PMMA), polycarbonates, polyethylenes, oxidized polyethylene, polypropylene, polyisobutylene, polystyrenes, poly(styrene)-co-(ethylene), polysulfones, polyethersulfones, polyarylsulfones, polyarylethers, polyolefins, polyacrylates, polyvinyl derivatives, cellulose derivatives, polyurethanes, polyamides, polyimides, polyesters, silicone resins, epoxy resins, polyvinyl alcohol, polyacrylic acid, and the like. Copolymer materials such as polystyrene-acrylonitrile, polyethylene-acrylate, vinylidenechloride-vinylchloride, vinylacetate-vinylidene chloride, styrene-alkyd resins are also examples of suitable binder materials. The copolymers may be block, random, or alternating copolymers. In some embodiments, polymethyl methacrylate or a polystyrene is the polymer binder, in terms of their cost and wide availability. The polymer binder, when used, has the role to provide a coating or film forming composition.

Phase change materials can also be used as the polymer binder. Phase change materials are known in the art, and include for example crystalline polyethylenes such as Polywax® 2000, Polywax® 1000, Polywax® 500, and the like from Baker Petrolite, Inc.; oxidized wax such as X-2073 and Mekon wax, from Baker-Hughes Inc.; crystalline polyethylene copolymers such as ethylene/vinyl acetate copolymers,

ethylene/vinyl alcohol copolymers, ethylene/acrylic acid copolymers, ethylene/methacrylic acid copolymers, ethylene/carbon monoxide copolymers, polyethylene-b-polyallyl-lylene glycol wherein the alkylene portion can be ethylene, propylene, butylenes, pentylene or the like, and including the polyethylene-b-(polyethylene glycol)s and the like; crystalline polyamides; polyester amides; polyvinyl butyral; polyacrylonitrile; polyvinyl chloride; polyvinyl alcohol hydrolyzed; polyacetal; crystalline poly(ethylene glycol); poly(ethylene oxide); poly(ethylene terephthalate); poly(ethylene succinate); crystalline cellulose polymers; fatty alcohols; ethoxylated fatty alcohols; and the like, and mixtures thereof.

In general, most any organic polymer can be used. However, in embodiments, because heat generated by the infrared absorber is used to erase the visible image, the polymer can be selected such that it has thermal properties that can withstand the elevated temperatures that may be used for erasing formed images based on the specific photochromic material that is chosen.

In embodiments, the imaging composition can be applied in one form, and dried to another form for use. Thus, for example, the imaging composition comprising photochromic material, infrared absorber, and solvent or polymer binder may be dissolved or dispersed in a solvent for application to or impregnation into a substrate, with the solvent being subsequently evaporated to form a dry layer.

In general, the imaging composition can include the carrier and imaging material in any suitable amounts, such as from about 5 to about 99.5 percent by weight carrier, such as from about 30 to about 70 percent by weight carrier, from about 0.05 to about 50 percent by weight photochromic material, such as from about 0.1 to about 5 percent photochromic material by weight, and from about 0.1 to about 30 percent by weight infrared absorber, such as from about 1 to about 10 percent infrared absorber by weight.

For applying the imaging layer to the image forming medium substrate, the image forming layer composition can be applied in any suitable manner. For example, the image forming layer composition can be mixed and applied with any suitable solvent or polymer binder, and subsequently hardened or dried to form a desired layer. Further, the image forming layer composition can be applied either as a separate distinct layer to the supporting substrate, or it can be applied so as to impregnate into the supporting substrate.

The image forming medium may comprise a supporting substrate, coated or impregnated on at least one side with the imaging layer. As desired, the substrate can be coated or impregnated on either only one side, or on both sides, with the imaging layer. When the imaging layer is coated or impregnated on both sides, or when higher visibility of the image is desired, an opaque layer may be included between the supporting substrate and the imaging layer(s) or on the opposite side of the supporting substrate from the coated imaging layer. Thus, for example, if a one-sided image forming medium is desired, the image forming medium may include a supporting substrate, coated or impregnated on one side with the imaging layer and coated on the other side with an opaque layer such as, for example, a white layer. Also, the image forming medium may include a supporting substrate, coated or impregnated on one side with the imaging layer and with an opaque layer between the substrate and the imaging layer. If a two-sided image forming medium is desired, then the image forming medium may include a supporting substrate, coated or impregnated on both sides with the imaging layer, and with at least one opaque layer interposed between the two coated imaging layers. Of course, an opaque supporting substrate,

such as conventional paper, may be used in place of a separate supporting substrate and opaque layer, if desired.

Any suitable supporting substrate may be used. For example, suitable examples of supporting substrates include, but are not limited to, glass, ceramics, wood, plastics, paper, fabrics, textile products, polymeric films, inorganic substrates such as metals, and the like. The plastic may be for example a plastic film, such as polyethylene film, polyethylene terephthalate, polyethylene naphthalate, polystyrene, polycarbonate, polyethersulfone. The paper may be, for example, plain paper such as XEROX® 4024 paper, ruled notebook paper, bond paper, silica coated papers such as Sharp Company silica coated paper, Jujo paper, and the like. The substrate may be a single layer or multi-layer where each layer is the same or different material. In embodiments, the substrate has a thickness ranging for example from about 0.3 mm to about 5 mm, although smaller or greater thicknesses can be used, if desired.

When an opaque layer is used in the image forming medium, any suitable material may be used. For example, where a white paper-like appearance is desired, the opaque layer may be formed from a thin coating of titanium dioxide, or other suitable material like zinc oxide, inorganic carbonates, and the like. The opaque layer can have a thickness of, for example, from about 0.001 mm to about 10 mm, such as about 0.1 mm to about 5 mm, although other thicknesses can be used.

If desired, a further overcoating layer may also be applied over the applied imaging layer. The further overcoating layer may, for example, be applied to further adhere the underlying layer in place over the substrate, to provide wear resistance, to improve appearance and feel, and the like. The overcoating layer can be the same as or different from the substrate material, although in embodiments at least one of the overcoating layer and substrate layer is clear and transparent to permit visualization of the formed image. The overcoating layer can have a thickness of, for example, from about 0.001 mm to about 10 mm, such as about 0.1 mm to about 5 mm, although other thicknesses can be used. For example, if desired or necessary, the coated substrate can be laminated between supporting sheets such as plastic sheets.

In embodiments where the imaging material is coated on or impregnated into the substrate, the coating can be conducted by any suitable method available in the art, and the coating method is not particularly limited. For example, the imaging material can be coated on or impregnated into the substrate by dip coating the substrate into a solution of the imaging material composition followed by any necessary drying, or the substrate can be coated with the imaging composition to form a layer thereof. Similarly, the protective coating can be applied by similar methods.

Where the photochromic material and infrared absorber are mixed with a solvent applied on the substrate, and where the solvent system is retained in the final product, additional processing may be required. As a result, where the photochromic material and infrared absorber are simply coated on the substrate, a cover material is generally applied over the solvent system to constrain the solvent system in place on the substrate. Thus, for example, the cover material can be a solid layer, such as any of the suitable materials disclosed above for the substrate layer. In an alternative embodiment, a polymer material or film may be applied over the photochromic material and infrared absorber, where the polymer film penetrates the photochromic material and infrared absorber at discrete points to in essence form pockets or cells of imaging material that are bounded on the bottom by the substrate and on the sides and top by the polymeric material. The height of the

cells can be, for example, from about 1 micron to about 1000 microns, although not limited thereto. The cells can be any shape, for example square, rectangle, circle, polygon, or the like. In these embodiments, the cover material is advantageously transparent and colorless, to provide the full color contrast effect provided by the photochromic material.

In another embodiment, the solvent system with the photochromic material and infrared absorber can be encapsulated or microencapsulated, and the resultant capsules or microcapsules deposited or coated on the substrate as described above. Any suitable encapsulation technique can be used, such as simple and complex coacervation, interfacial polymerization, in situ polymerization, phase separation processes. For example, a suitable method if described for ink materials in U.S. Pat. No. 6,067,185, the entire disclosure of which is incorporated herein by reference and can be readily adapted to the present disclosure. Useful exemplary materials for simple coacervation include gelatin, polyvinyl alcohol, polyvinyl acetate and cellulose derivatives. Exemplary materials for complex coacervation include gelatin, acacia, acra-geenan, carboxymethylcellulose, agar, alginate, casein, albumin, methyl vinyl ether-co-maleic anhydride. Exemplary useful materials for interfacial polymerization include diacyl chlorides such as sebacoyl, adipoyl, and di or poly-amines or alcohols and isocyanates. Exemplary useful materials for in situ polymerization include for example polyhydroxyamides, with aldehydes, melamine or urea and formaldehyde; water-soluble oligomers of the condensate of melamine or urea and formaldehyde, and vinyl monomers such as for example styrene, methyl methacrylate and acrylonitrile. Exemplary useful materials for phase separation processes include polystyrene, polymethylmethacrylate, polyethylmethacrylate, ethyl cellulose, polyvinyl pyridine and polyacrylonitrile. In these embodiments, the encapsulating material is also transparent and colorless, to provide the full color contrast effect provided by the photochromic material.

Where the photochromic material and infrared absorber are encapsulated, the resultant capsules can have any desired average particle size. For example, suitable results can be obtained with capsules having an average size of from about 2 to about 1000 microns, such as from about 10 to about 600 or to about 800 microns, or from about 20 to about 100 microns, where the average size refers to the average diameter of the microcapsules and can be readily measured by any suitable device such as an optical microscope. For example, in embodiments, the capsules are large enough to hold a suitable amount of photochromic material to provide a visible effect when in the colored form, but are not so large as to prevent desired image resolution.

In its method aspects, the present disclosure involves providing an image forming medium comprised of a substrate and an imaging layer comprising a photochromic material and infrared absorber dispersed in a solvent or polymeric binder, wherein the imaging composition is imageable by light and erasable in a short time period by a combination of light and infrared radiation, and exhibits a reversible transition between a colorless and a colored state. To provide separate writing and erasing processes, imaging is conducted by applying a first stimulus, such as UV light irradiation, to the imaging material to cause a color change, and erasing is conducted by applying a second, different stimulus, such as a combination of visible light and infrared irradiation, to the imaging material to reverse the color change in a short time period. Thus, for example, the imaging layer as a whole could be sensitive at a first (such as UV) wavelength that causes the photochromic material to convert from a clear to a colored state, while the imaging layer as a whole could be sensitive at

a second, different (such as visible) wavelength and to heat that causes the photochromic material to convert from the colored back to the clear state in a short time period.

In a writing process, the image forming medium is exposed to an imaging light having an appropriate activating wavelength, such as a UV light source such as a light emitting diode (LED), in an imagewise fashion. The imaging light supplies sufficient energy to the photochromic material to cause the photochromic material to convert, such as isomerize, from a clear state to a colored state to produce a colored image at the imaging location, and for the photochromic material to isomerize to stable isomer forms to lock in the image. The amount of energy irradiated on a particular location of the image forming medium can affect the intensity or shade of color generated at that location. Thus, for example, a weaker intensity image can be formed by delivering a lesser amount of energy at the location and thus generating a lesser amount of colored photochromic unit, while a stronger intensity image can be formed by delivering a greater amount of energy to the location and thus generating a greater amount of colored photochromic unit. When suitable photochromic material, solvent or polymer binder, and irradiation conditions are selected, the variation in the amount of energy irradiated at a particular location of the image forming medium can thus allow for formation of grayscale images, while selection of other suitable photochromic materials can allow for formation of full color images.

Once an image is formed by the writing process, the formation of stable isomer forms of the photochromic material within the imaging materials locks in the image. That is, the isomer forms of the selected photochromic materials are more stable to ambient heat and light, and thus exhibit greater long-term stability. The image is thereby "frozen" or locked in, and cannot be readily erased in the absence of a specific second stimuli such as heat and light, particularly in a short time period. In embodiments, the image is locked in, and cannot be readily erased by ambient heat or light alone, and requires elevated temperature and light in order to revert back to the colorless state. The imaging substrate thus provides a reimagineable substrate that exhibits a long-lived image life-time, but which can be erased as desired and reused for additional imaging cycles.

In an erasing process, the writing process is essentially repeated, except that a different stimuli, such as a different wavelength irradiation light, such as visible light and infrared irradiation. The infrared absorber absorbs the infrared radiation, and locally heats the imaging material. The erasing process causes the isomerizations to reverse and the photochromic unit to convert, such as isomerize, from a colored state to a clear state to erase the previously formed image at the imaging location in a short time period. The erasing procedure can be on an image-wise fashion or on the entire imaging layer as a whole, as desired.

The different stimuli, such as different light irradiation wavelengths, can be suitably selected to provide distinct writing and erasing operations. For example, in one embodiment, the photochromic material is selected to be sensitive to UV light to cause isomerization from the clear state to the colored state, but to be sensitive to visible light and heat to cause isomerization from the colored state to the clear state. In other embodiments, the writing and erasing wavelengths are separated by at least about 10 nm, such as at least about 20 nm, at least about 30 nm, at least about 40 nm, at least about 50 nm, or at least about 100 nm. Thus, for example, if the writing wavelength is at a wavelength of about 360 nm, then the erasing wavelength is desirably a wavelength of greater than 400 nm or greater than about 500 nm. Of course, the relative

separation of sensitization wavelengths can be dependent upon, for example, the relatively narrow wavelengths of the exposing apparatus.

The separate imaging lights used to form the transient image and erase the transient image may have any suitable predetermined wavelength scope such as, for example, a single wavelength or a band of wavelengths. In various exemplary embodiments, the imaging lights are an ultraviolet (UV) light and a visible light each having a single wavelength or a narrow band of wavelengths. For example, the UV light can be selected from the UV light wavelength range of about 200 nm to about 475 nm, such as a single wavelength at about 365 nm or a wavelength band of from about 360 nm to about 370 nm. For forming the image, as well as for erasing the image, the image forming medium may be exposed to the respective imaging or erasing light for a time period ranging from about 10 milliseconds to about 5 minutes, particularly from about 30 milliseconds to about 1 minute. The imaging light may have an intensity ranging from about 0.1 mW/cm<sup>2</sup> to about 100 mW/cm<sup>2</sup>, particularly from about 0.5 mW/cm<sup>2</sup> to about 10 mW/cm<sup>2</sup>.

The erasing light is strong visible light and a separate or combined strong infrared light of a wavelength which overlaps with the absorption spectrum of the colored state isomer in the visible region. For example the erasing useful light may have a wavelength ranging from about 400 nm to about 800 nm or more preferably from about 500 nm to about 800 nm. The usable visible light of the erasing may be obtained from a Xenon light source with a bulb having a power from 5 W to about 1000 W or more preferably from about 20 W to about 200 W, which is placed in the proximity of the areas of the document which is to be erased. Another suitable erasing light source is an LED having a wavelength in the visible region of the light spectrum, as defined above. The erasing light may be having a single wavelength or a narrow band of wavelengths.

In various exemplary embodiments, imaging light corresponding to the predetermined image may be generated for example by a computer or a Light Emitting Diode (LED) array screen and the image is formed on the image forming medium by placing the medium on or in proximity to the LED screen for the desired period of time. In other exemplary embodiments, a UV Raster Output Scanner (ROS) may be used to generate the UV light in an image-wise pattern. This embodiment is particularly applicable, for example, to a printer device that can be driven by a computer to generate printed images in an otherwise conventional fashion. That is, the printer can generally correspond to a conventional inkjet printer, except that the inkjet printhead that ejects drops of ink in the imagewise fashion can be replaced by a suitable UV light printhead that exposes the image forming medium in an imagewise fashion. In this embodiment, the replacement of ink cartridges is rendered obsolete, as writing is conducted using a UV light source. The printer can also include a heating device, which can be used to apply heat to the imaging material to erase any existing images. Other suitable imaging techniques that can be used include, but are not limited to, irradiating a UV light onto the image forming medium through a mask, irradiating a pinpoint UV light source onto the image forming medium in an imagewise manner such as by use of a light pen, and the like.

For erasing an image in order to reuse the imaging substrate, in various exemplary embodiments, the substrate can be exposed to a suitable imaging light and heat, to cause the image to be erased. Such erasure can be conducted in any suitable manner, such as by exposing the entire substrate to the erasing light and heat at once, exposing the entire substrate to the erasing light and heat in a successive manner such

as by scanning the substrate, or the like. In other embodiments, erasing can be conducted at particular points on the substrate, such as by using a light pen and focused heat source, or the like.

According to various exemplary implementations, the color contrast that renders the image visible to an observer may be a contrast between, for example two, three or more different colors. The term "color" may encompass a number of aspects such as hue, lightness and saturation, where one color may be different from another color if the two colors differ in at least one aspect. For example, two colors having the same hue and saturation but are different in lightness would be considered different colors. Any suitable colors such as, for example, red, white, black, gray, yellow, cyan, magenta, blue, and purple, can be used to produce a color contrast as long as the image is visible to the naked eye of a user. However, in terms of desired maximum color contrast, a desirable color contrast is a dark gray or black image on a light or white background, such as a gray, dark gray, or black image on a white background, or a gray, dark gray, or black image on a light gray background.

In various exemplary embodiments, the color contrast may change such as, for example, diminish during the visible time, but the phrase "color contrast" may encompass any degree of color contrast sufficient to render an image discernable to a user regardless of whether the color contrast changes or is constant during the visible time.

An example is set forth hereinbelow and is illustrative of different compositions and conditions that can be utilized in practicing the disclosure. All proportions are by weight unless otherwise indicated. It will be apparent, however, that the disclosure can be practiced with many types of compositions and can have many different uses in accordance with the disclosure above and as pointed out hereinafter.

## EXAMPLES

### Example 1

A photochromic material, a methoxy substituted dithienylethene, is synthesized according to the procedure described in "Dithienylethenes with a Novel Photochromic Performance", J. Org. Chem., 2002, 67, 4574-4578.

A solution is made by dissolving 140 mg of the photochromic material and 50 mg of IR 895, which is an infrared absorber commercially available from Sigma-Aldrich, in 5 ml of a solution of polymethylmethacrylate (PMMA, polymeric binder) dissolved in toluene and tetrahydrofuran as solvent (PMMA/Solvent=20 g/100 ml). The solution is then spin-coated onto quartz slides (1000 rpm; 60 seconds). The coated slides are allowed to dry, to provide a reimageable media, ready for printing.

Initially, the slides are clear (no image base present). Exposure to UV light at a wavelength of 365 nm from a UV LED printbar generates a visible image. The printed image is stable against ambient exposure on the paper. However, exposure to a combination of visible light and infrared radiation provided from a Quartz tube model QRT from Chromalox erases the image in about 5 seconds.

Comparison test samples are made in a similar way except that no IR absorber is used. The samples erase in longer time than the sample containing IR absorbing dye. The composition can be re-imaged and re-erased as necessary.

It will be appreciated that various of the above-disclosed and other features and functions, or alternatives thereof, may be desirably combined into many other different systems or applications. Also that various presently unforeseen or unan-

ticipated alternatives, modifications, variations or improvements therein may be subsequently made by those skilled in the art which are also intended to be encompassed by the following claims.

5 What is claimed is:

1. An image forming medium, comprising a substrate; and an imaging layer coated on or impregnated into said substrate, wherein the imaging layer comprises an imaging composition comprising a photochromic or photochromic-thermochromic material and an infrared absorber dissolved or dispersed in a solvent or polymeric binder; wherein: the photochromic or photochromic-thermochromic material and the infrared absorber are selected so that: the infrared absorber absorbs infrared light of a wavelength in a range from about 730 nm to about 1500 nm; the imaging composition is imageable by light of a first wavelength and erasable in a short time period by a combination of infrared radiation and light of a second wavelength, and exhibits a reversible transition between a colorless and a colored state; and the short time period is the time period for the maximum absorbance of the imaging composition in the region 400-800 nm to be reduced from its initial absorbance to one half of the initial absorbance, in about 10 seconds or less.

30 2. The image forming medium of claim 1, wherein the photochromic or photochromic-thermochromic material and the infrared absorber are selected so that the image is readable for more than two days after imaging and storage at ambient temperature and under ambient light conditions.

35 3. The image forming medium of claim 1, wherein the infrared absorber absorbs and converts infrared radiation into heat to heat the photochromic or photochromic-thermochromic material.

40 4. The image forming medium of claim 1, wherein the infrared absorber is selected from the group consisting of infrared dyes, near infrared dye, analogs of infrared dyes, and analogs of near infrared dye.

45 5. The image forming medium of claim 1, wherein the infrared absorber is selected from the group consisting of aminium-salt-based compounds described by formula (1) and diimmonium-salt-based compounds described by formula (2):

(1)



(2)



60 wherein  $\text{R}_1$ ,  $\text{R}_2$ ,  $\text{R}_3$ , and  $\text{R}_4$  each independently represent hydrogen atom, alkyl group, substitution alkyl group, cyclic alkyl group, alkenyl group, alalkyl group or substituted alalkyl group, and  $\text{X}^-$  denotes a suitable negative ion.

65 6. The image forming medium of claim 1, wherein the infrared absorber is selected from the group consisting of indocyanine green, fluorescein isothiocyanate, rhodamine,

23

phycoerythrin, phycocyanin, allophycocyanin, o-phthaldehyde, fluorescamine, Rose Bengal, trypan blue, and fluoro-gold.

7. The image forming medium of claim 1, wherein the infrared absorber does not significantly affect the hue of the imaging composition. 5

8. The image forming medium of claim 1, wherein the photochromic or photochromic-thermochromic material is selected from the group consisting of spiropyrans, diethiethenes, naphthopyrans, chromenes, and fulgides, and 10 mixtures thereof.

9. The image forming medium of claim 1, wherein the photochromic material is an alkoxy substituted dithiethene represented by the formula: 15



wherein each R, which can be the same or different represents an unsubstituted or substituted, straight, branched, or cyclic, 30 alkyl group having from 1 to about 20 carbon atoms, an unsubstituted or substituted aryl group having from about 6 to about 30 carbon atoms, an unsubstituted or substituted arylalkyl group having from about 7 to about 50 carbon atoms, silyl groups, nitro groups, cyano groups, halide atoms, amine groups, hydroxy groups, alkoxy groups having from 1 to about 50 carbon atoms, aryloxy groups having from about 6 to about 30 carbon atoms, alkylthio groups having from 1 to about 50 carbon atoms, arylthio groups having from about 6 to about 30 carbon atoms, aldehyde groups, ketone groups, 35 ester groups, amide groups, carboxylic acid groups, and sulfonic acid groups.

10. The image forming medium of claim 9, wherein the alkyl group is substituted by one or more groups selected from the group consisting of silyl groups, nitro groups, cyano groups, halide atoms, amine groups, hydroxy groups, alkoxy groups, aryloxy groups, alkylthio groups, arylthio groups, 45 aldehyde groups, ketone groups, ester groups, amide groups, carboxylic acid groups, and sulfonic acid groups.

11. The image forming medium of claim 1, wherein the photochromic material is represented by the general formula 50 (I)



wherein:

each X independently represents hydrogen, an alkyl chain 65 having 1 to 20 carbon atoms, bromine, chlorine or an iodine atom,

24

A represents a group of formula (a)-(c), and B represents a group of formula (d)-(f),



[a]



[b]



[c]



[d]



[e]



[f]

wherein:

R<sub>4</sub> represents an aryloxy group, a substituted and unsubstituted heteroaromatic group, an alkoxy group, or a substituted alkoxy group, where the alkyl portion of the alkoxy group represents a straight, branched or cyclic, substituted or unsubstituted, alkyl group of from 1 to about 40 carbon atoms,

R<sub>5</sub> represents an aryl group, a substituted or unsubstituted alkylaryl group wherein hetero atoms either may or may not be present in the alkyl portion of the alkylaryl group or the aryl portion of the alkylaryl group, a cyano group, a carboxylic acid group, or an unsaturated alkene group,

R<sub>6</sub> represents a hydrogen atom, an alkyl group, a halogen atom, an alkoxy group, a fluoroalkyl group, a cyano group, an aryl group, or a substituted alkylaryl group,

R<sub>7</sub> represents an alkyl group, an aryl group, an alkylaryl group including substituted alkylaryl groups, unsubstituted alkylaryl groups, and wherein hetero atoms either may or may not be present in the alkyl portion of the alkylaryl group or the aryl portion of the alkylaryl,

R<sub>8</sub> represents an aryloxy group, substituted and unsubstituted heteroaromatic group, or an alkoxy group or substituted alkoxy group where the alkyl portion of the alkoxy group represents a straight, branched or cyclic, substituted or unsubstituted, alkyl group of from 1 to about 40 carbon atoms,

25

$R_9$  represents an aryl group, a substituted or unsubstituted alkylaryl group wherein hetero atoms either may or may not be present in the alkyl portion of the alkylaryl group or the aryl portion of the alkylaryl group, a cyano group, a carboxylic acid group, or an unsaturated alkene group,

$R_{10}$  represents a hydrogen atom, an alkyl group, a halogen atom, an alkoxy group, a fluoroalkyl group, a cyano group, an aryl group, or a substituted alkylaryl group,

$R_{11}$  represents an alkyl group, an aryl group, or a substituted or unsubstituted alkylaryl group wherein hetero atoms either may or may not be present in the alkyl portion of the alkylaryl group or the aryl portion of the alkylaryl group, and

U and Z each independently represent sulfur or oxygen atoms.

12. The image forming medium of claim 1, wherein the photochromic material is represented by the general formulae (II), (III), (IV), (V), (VI), (VII)



wherein:

$R_1$ ,  $R_2$  are each independently selected from substituted alkyl groups, unsubstituted alkyl groups, linear alkyl groups, and branched alkyl groups, and wherein hetero atoms either may or may not be present in the alkyl group, a halogen group, an alkoxy group, a cyano group, a nitro group, an amino group, an amide group, an aryl

60

[VII] 55

65

26

group, and an alkylaryl group wherein hetero atoms either may or may not be present in the alkyl portion of the alkylaryl group or the aryl portion of the alkylaryl group,

5 in formula (II), X represents S or O,

in formula (IV), X represents S, O or  $C=O$ , and Y represents O,  $CH_2$  or  $C=O$ ,

in formula (V), Y represents  $CH_2$  or  $C=O$ ,

in formula (VI), X represents CH or N, and

in formula (VII), Y represents  $CH_2$  or  $C=O$ ,

and wherein:

A represents a group of formula (a)-(c), and

B represents a group of formula (d)-(f),

[a]



[b]



[c]



[d]



[e]



[f]



wherein:

$R_4$  represents an aryloxy group, a substituted and unsubstituted heteroaromatic group, an alkoxy group, or a substituted alkoxy group, where the alkyl portion of the alkoxy group represents a straight, branched or cyclic, substituted or unsubstituted, alkyl group of from 1 to about 40 carbon atoms,

$R_5$  represents an aryl group, a substituted or unsubstituted alkylaryl group wherein hetero atoms either may or may not be present in the alkyl portion of the alkylaryl group or the aryl portion of the alkylaryl group, a cyano group, a carboxylic acid group, or an unsaturated alkene group,

$R_6$  represents a hydrogen atom, an alkyl group, a halogen atom, an alkoxy group, a fluoroalkyl group, a cyano group, an aryl group, or a substituted alkylaryl group,

27

$R_7$  represents an alkyl group, an aryl group, an alkylaryl group including substituted alkylaryl groups, unsubstituted alkylaryl groups, and wherein hetero atoms either may or may not be present in the alkyl portion of the alkylaryl group or the aryl portion of the alkylaryl,

$R_8$  represents an aryloxy group, substituted and unsubstituted heteroaromatic group, or an alkoxy group or substituted alkoxy group where the alkyl portion of the alkoxy group represents a straight, branched or cyclic, substituted or unsubstituted, alkyl group of from 1 to about 40 carbon atoms,

$R_9$  represents an aryl group, a substituted or unsubstituted alkylaryl groups wherein hetero atoms either may or may not be present in the alkyl portion of the alkylaryl group or the aryl portion of the alkylaryl group, a cyano group, a carboxylic acid group, or an unsaturated alkene group,

$R_{10}$  represents a hydrogen atom, an alkyl group, a halogen atom, an alkoxy group, a fluoroalkyl group, a cyano group, an aryl group, or a substituted alkylaryl group,

$R_{11}$  represents an alkyl group, an aryl group, or a substituted or unsubstituted alkylaryl group wherein hetero atoms either may or may not be present in the alkyl portion of the alkylaryl group or the aryl portion of the alkylaryl, and

U and Z each independently represent sulfur or oxygen.

**13.** The image forming medium of claim 1, wherein the photochromic material is dispersed in a polymer selected from the group consisting of polyalkylacrylates, polycarbonates, polyethylenes, oxidized polyethylene, polypropylene, polyisobutylene, polystyrenes, poly(styrene)-co-(ethylene), polysulfones, polyethersulfones, polyarylsulfones, polyarylethers, polyolefins, polyacrylates, polyvinyl derivatives, cellulose derivatives, polyurethanes, polyamides, polyimides, polyesters, silicone resins, epoxy resins, polyvinyl alco-

28

hol, polyacrylic acid, polystyrene-acrylonitrile, polyethylene-acrylate, vinylidenechloride-vinylchloride, vinylacetate-vinylidene chloride, styrene-alkyd resins, and mixtures thereof.

**14.** The image forming medium of claim 1, wherein the photochromic material is dissolved in a solvent selected from the group consisting of straight chain aliphatic hydrocarbons, branched chain aliphatic hydrocarbons, aromatic, halogenated, polar solvents, and mixtures thereof.

**15.** The image forming medium of claim 1, wherein the photochromic or photochromic-thermochromic material is present in an amount of from about 0.01% to about 20% by weight of a total weight of the imaging composition, and the infrared absorber is present in an amount of from about 0.1 to about 30 percent by weight of a total weight of the imaging composition.

**16.** The image forming medium of claim 1, wherein the substrate is selected from the group consisting of glass, ceramic, wood, plastic, paper, fabric, textile, metals, plain paper, and coated paper.

**17.** The image forming medium of claim 1, wherein the solvent mixture is provided in the form of encapsulated amounts of the solvent mixture.

**18.** A system for imaging the image forming medium of claim 1, the system comprising:

a printer comprising an imaging member that outputs the first wavelength and an erase component that outputs infrared radiation and the second wavelength, that is capable of heating and flooding the image forming medium with heat and light of the second wavelength simultaneously.

**19.** The image forming medium of claim 1, wherein the first wavelength is from 200 to 500 nanometers and the second wavelength is from 501 to 800 nanometers.

\* \* \* \* \*